

## UNITED STATES PATENT OFFICE

2,033,163

PROCESS OF DEPILATING AND BATING  
HIDES AND A BATE FOR THESE PURPOSES

Leo Wallerstein, New York, and Julius Pfannmuller, Stapleton, N. Y., assignors to Wallerstein Company, Inc., New York, N. Y., a corporation of New York

No Drawing. Application May 25, 1932, Serial No. 613,546. Renewed June 8, 1935

12 Claims. (Cl. 149—3)

This invention relates to an improved method or process of treating hides and skins prior to tanning, and to an improved bate suitable for carrying out the invention.

5 Hides and skins before they are tanned or converted into commercial leather have to be subjected to various processes. After the skin has been tanned, it is generally cured or preserved. In order to bring the cured or otherwise preserved skins or hides to a condition closely approximating the natural state they are subjected to a soaking process, that is, this soaking process effects a softening of the skin. This is usually carried out by washing and permitting the skins to lie in 10 water, with or without the addition of certain chemical or enzymatic substances for varying times, as from a few hours to a few days.

15 After the hides or skins have been soaked to the desired extent, the hides are treated so that they can be dehaired, the hair of the hides being loosened so that it can be easily removed by various dehairing methods. The process commonly used for loosening the hair consists in soaking the skins or hides in lime solutions or lime solutions 20 to which sulfides, such as sodium sulfide, red arsenic or other chemicals have been added. It has also been proposed to effect the loosening of the hair of the hides or skins by certain enzymatic methods, such use of enzymes being usually carried out after the skins have been first subjected to what is known as an alkaline bath. After the 25 hides or skins have been subjected to the lime or alkaline process, they are usually partly neutralized and then subjected to a bating or puering process.

30 In carrying out this particular method of bating, the hides or skins are neutralized to a pH ranging from a slight acidity to about 10, and this lessening of the alkalinity is achieved by the addition of a suitable acid, suitable acid salts or ammonia salts, and neutralizing agents may also be formed by a bacterial action, as, for instance, by the formation or production of lactic, acetic or butyric acids.

35 Bating baths have been suggested containing proteolytic enzymes which act on certain of the constituents of the hides or skins. The enzymes or enzymatic products used for this bathing bath may be derived from various sources, as, for instance, from pancreas glands or from preparations which contain the proteases of various plants or molds, or other micro-organisms, as, for instance, bacterial proteases.

40 This bathing or puering process, to which the 45 hides are subjected, is used to soften the hides

and get the hides in proper condition for tanning so that the resulting leather is of the desired quality. Where the skins or hides are dehaired by the use of proteolytic enzymes, the special bathing methods above referred to are not as a rule necessary, the bathing or conditioning of the hides or skins taking place simultaneously with the loosening of the hair, so that when the hide is dehaired it has also been suitably bated or softened, and this method of dehairing and bathing may be carried out at the same time and in the same bath.

45 Whatever the process employed, however, the hides or skins after the dehairing and bathing or puering should have a soft or flaccid feel and should be sufficiently soft so that, as a rough 50 test, they will retain the impression of a thumb print, the softness depending upon the kind of finished leather desired, and the hides and skins should have a clean and low grain, by which is meant the pores of the skins should be as fine as possible and flattened out so that the grain feels very smooth; in other words, the grain should be the opposite of what is known as a "goose flesh effect".

55 It is very desirable, if not essential, that in the production of a finished leather having the desired fineness or tightness of the grain that this condition of the hide or skin should be produced prior to the tanning process, that is, during the dehairing and bathing processes. We have discovered that the desired grain condition and consequent improvement in the finished leather can be obtained by treating the hides and skins, during the above mentioned methods or any of them, with comparatively small amounts of water soluble organic substances which have in their chemical constitution the group represented by the general formula



40

that is, the acidamide group, for instance, such substances as acetamide, urea, semi-carbazide, salts of carbamic acid, biuret or other derivatives of substances wherein, in the group,



45

50 one or both hydrogens are substituted by an alkyl or phenyl group, for instance, acetanilide.

55 A particular feature of the present invention resides in the fact that the treatment with the

carbonylamido compound is carried out in a medium or bath in which putrefaction or fermentation does not take place, as such putrefaction or fermentation would decrease and destroy the carbonyl-amido compound and/or prevent it from exerting its beneficial action.

Another feature of the present invention resides in the fact that the action of the carbonyl-amido compound is most effectively obtained 10 when the compound is utilized in very small quantities usually less than 1% in the bath.

The amounts of these substances needed for the above described purpose are relatively small and can be varied greatly, depending on the effect 15 desired. As a general rule, 1 part in 200 to 1 part in 1000 parts of the bath in which the skins are treated will be sufficient to give good effects. These substances may be applied either in a separate bath at any of the above mentioned stages 20 prior to tanning, or by adding these substances in the proper proportions to a bath which is used in the above processes. For instance, these substances can be used by adding the same during the soaking process, or the skins after the soaking 25 process may be treated in a bath containing the above mentioned substances. The skins may also be subjected to accomplish the purpose of this invention after they have been subjected to the lime or lime and sulfide dehairing bath.

30 We have found that a very good method and one which has given excellent results is the one in which we use these substances in connection with the bathing process, or in case the hides are dehaired with an enzymatic unhaired process, 35 by adding same to the enzymatic dehairing bath. Substantially the same results are obtained by using a separate bath subsequent to the bathing or enzymatic dehairing and using a bath which contains any or a mixture of the above mentioned 40 substances in the proper proportions.

The action of these substances is particularly pronounced on the condition of the grain of the hide or skin. We have found that by treating the hides or skins as set forth the grain becomes 45 smoother, tighter, and the appearance of the finished leather is far superior and of better quality than of leather which is finished and tanned in which the treatment with these substances has been omitted. For certain kinds of 50 leather, for instance, in the treatment of heavy hide, as in the manufacture of sole leather, we have found that proteolytic enzymes for bathing or puering may be greatly reduced or even dispensed with entirely when using a bath containing 55 the above substances. As a general rule, however, we have found that by combining the good effect of the above mentioned substances together with a proper bathing, such as is done by means of proteolytic enzymes, the best results 60 are obtained. For such a procedure it is advisable, as mentioned above, to use these substances in the same bath with the proteolytic enzyme bath or at a stage shortly before or shortly subsequent to the bathing process. Many substances 65 belonging to the above mentioned groups and suitable for the purpose of the invention are now available in technical pure form, for instance, urea or acetanilide.

As examples of carrying out our invention, the 70 following may be given:

Example No. 1.—1000 lbs. calf skins are soaked and then unhaired as it is usually done, by means of a lime bath containing sodium sulfide. The skins are washed and then brought into a bath 75 containing 1 to 5 parts urea to 2000 parts water

and left therein for a few hours, or if more desirable, overnight, in which case it is preferable to add a suitable disinfectant. After this treatment, the skins may be subjected to a desired bathing treatment and are finished as desired.

Example No. 2.—1000 lbs. dry goat skins are soaked, limed and unhaired as usual. They are partially neutralized and bathed in a bath containing a proteolytic enzymatic bathing preparation, such as a pancreas preparation, or an enzyme preparation of bacterial origin. To this bathing bath there are added 1/2 to 2 lbs. of acetanilide or urea for each 1000 lbs. of bathing liquor. The bathing is carried out as desired, and the skins finished in any desired way.

Example No. 3.—1000 lbs. dry weight goat skins are soaked and unhaired in the customary lime bath. They then are puered in the usual way with a dog dung infusion. After the puering they are washed and brought into a bath containing 20 from 1 to 5 parts of urea or acetamide or a mixture of both in 1000 parts of water and left therein for a sufficient time, for instance, a few hours or overnight. If the time is longer than a few hours, the addition of a disinfectant is recommended.

Example No. 4.—1000 lbs. goat skins are soaked as usual and subjected to an alkaline swelling bath containing caustic soda. After this the skins are partly neutralized and subjected to the 30 influence of an enzymatic dehairing bath containing proteases of bacterial origin. A disinfectant is added to this dehairing bath; 10 parts urea are added for 5000 parts of the dehairing bath. After the dehairing, the skins are tanned 35 and finished as desired.

Example No. 5.—1000 lbs. goat skins are soaked as usual and subjected to an alkaline bath containing caustic soda. After the skins are partly neutralized they are subjected to a dehairing bath 40 produced by the addition of an enzymatic liquor of bacterial origin to which a disinfectant has been added. After the hair has been loosened and the skins have been unhaired, they are brought into a bath containing from 2 to 10 parts 45 of urea or 2 to 10 parts of the ammonium salt of carbaminic acid to 5000 parts of water and are left in this bath long enough until the grain has been brought into the required condition; as a rule a few hours is sufficient time. They are 50 then finished as usual.

Example No. 6.—Sheep skins are painted on the flesh side with a preparation containing dehairing enzymes of bacterial origin. To these preparations, approximately 1% by weight of 55 acetamide are added. After dewooling, the skins are finished in the usual way. Of course, the amount of acetamide added for this purpose may vary in a wide range and instead of acetamide any other substances of the above mentioned 60 groups can be used.

In all the above examples the final leather will be of better quality and will especially show a finer and tighter grain than if the treatment with the above mentioned substances were 65 omitted.

The invention also contemplates the use of a novel bate which may be supplied to tanners or other workers in hides and skins and which may be used in the above described processes or 70 in variations of them.

Such bates may have different compositions, depending on the particular treatment to which the hides or skins are subjected, and we will give examples of bates which give good results.

Example A.—A mixture containing:

|                                                                | Per cent |
|----------------------------------------------------------------|----------|
| Urea.....                                                      | 15       |
| Pancreatin U. S. P.....                                        | 10       |
| 5 Inert substances such as wood flour or infusorial earth..... | 75       |

Example B.—A mixture containing:

|                                                                 | Pounds |
|-----------------------------------------------------------------|--------|
| Urea.....                                                       | 20     |
| 10 Acetanilide.....                                             | 10     |
| Ammonium chloride.....                                          | 60     |
| Dried pancreas gland.....                                       | 1-10   |
| 15 Inert substances such as wood flour or infusorial earth..... | 1-10   |

15 Instead of the U. S. P. pancreatin as in Example A, a corresponding amount of pancreas gland or pancreas extract may be used, or a protease preparation may be employed, such as is produced by the cultivation of molds, or proteases of bacterial origin, which are of required strength.

While a filler is preferably used as given in the examples, this may be omitted if desired.

25 It will also be understood that instead of ammonium chloride, as given in Example B, other deliming agents such as sodium bi-sulfite, ammonium sulfate, boric acid, or mixtures of these substances may be employed.

30 While the invention has been described in its preferred form, and in accordance with the best practice now known to us, it will be understood that the invention is not to be limited precisely to this and may be varied in some particulars and that the examples given are merely illustrative.

What is claimed is:

1. A process of treating hides and skins to produce an improved leather, which consists in bating the hides or skins prior to tanning in a bath containing a proteolytic enzymatic preparation and organic substances having the group



45 said substance being utilized in the amount of not more than 1% by weight in a non-putrefactive medium.

50 2. A process of treating hides and skins to produce an improved leather, which consists in bating the hides or skins prior to tanning in a bath containing a proteolytic enzymatic preparation and a relatively small amount of urea, said urea being utilized in amount less than 1% in a medium devoid of complex organic mixtures which give rise to putrefaction.

55 3. A process of treating hides and skins to produce an improved leather, which consists in treating the hides or skins prior to tanning in a bath containing a relatively small amount of acetanilide.

60 4. A process of treating hides and skins to produce an improved leather, which consists in treating the hides or skins prior to tanning in a bath containing a relatively small amount of acetanilide and urea.

5. The process of treating hides and skins to

produce an improved leather, which consists in treating the hides and skins prior to tanning in a bathing bath containing organic substances having the group



5

wherein one or both hydrogens are substituted by an alkyl or phenyl group.

6. The process of treating hides and skins to produce an improved leather, which consists in subjecting them to a bath containing a proteolytic enzyme and a substance having the group



15

said substance being utilized in the amount of not more than 1% by weight in a non-putrefactive medium.

7. The process of treating hides and skins to produce an improved leather, which consists in subjecting them to a bath containing a proteolytic enzyme and a substance having the group



25

wherein one or both hydrogens are substituted by an alkyl or phenyl group.

8. A bating preparation containing organic substances having the group



30

35 and a proteolytic enzyme, said organic substances being utilized in amounts less than 1% by weight in a non-putrefactive medium.

9. A bating preparation containing organic substances having the group



40

45 and a deliming agent, said organic substances being utilized in amounts less than 1% by weight in a non-putrefactive medium.

10. A bating preparation containing organic substances having the group



50

55 a proteolytic enzyme, and deliming agents, said organic substances being utilized in amounts less than 1% by weight in a non-putrefactive medium.

11. A bating preparation containing urea, and a protease, said preparation being utilized in a bath devoid of complex organic mixtures which give rise to putrefaction.

12. A bating preparation containing urea, a protease, and an ammonium salt, said preparation being utilized in a bath devoid of complex organic mixtures which give rise to putrefaction.

LEO WALLERSTEIN.  
JULIUS PFANNMULLER.